

# UNITED STATES PATENT OFFICE.

KURT HARING, OF HERSFELD, HESSE-NASSAU, GERMANY, ASSIGNOR TO THE CORPORATION OF ANHYDAT-LEDER-WERKE AKTIENGESELLSCHAFT, OF HERSFELD, GERMANY.

## PROCESS FOR TANNING OR IMPREGNATING HIDES.

1,285,144.

Specification of Letters Patent. Patented Nov. 19, 1918.

No Drawing.

Application filed February 16, 1916. Serial No. 78,581.

To all whom it may concern:

Be it known that I, KURT HARING, citizen of the German Empire, and resident of Hersfeld, Hesse-Nassau, Germany, with the post-office address Hainstrasse 14, have invented new and useful Improvements in Processes for Tanning or Impregnating Hides, of which the following is a specification.

10 My invention relates to improvements in tanning or impregnating hides by means of viscous substances, especially bituminous substances as for instance natural or artificial asphaltum or the like.

15 I have found that it is possible to use such bodies with great success as means for impregnating hides when the treatment is effected *in vacuo*. It is essential to have the hides to be impregnated well dried before; 20 this drying process may be effected in the manner described in the United States Patent No. 1,200,146, dated October 3, 1916, for the manufacture of leather products resembling leather, issued to Werner Spalteholz and 25 myself, that is to say by a treatment with liquids that have an attraction for water as for instance alcohol, acetone or their homologues.

30 I have found that it is impossible to impregnate hides with substances of a strong viscous nature by merely placing them in a molten mass.

35 Although it seems to be obvious, to raise the liquidity of the molten mass by raising the temperature, this could not be done as temperatures, that exceed 95°-100° C. are injurious to animal hides.

40 For this reason it was necessary to make use of the so called "diffusion process," which consists in filling the hides first with a solution and then treating the same by a molten mass, the latter being soluble in the solvent used before.

45 Now it has been found, that this procedure may be dispensed with by the process, which forms the subject of the present application.

50 According to my invention the hides are dehydrated and when completely dry placed into a closed receptacle. The air in this receptacle is then evacuated and the molten mass is introduced while a high vacuum is maintained continuously. As soon as the

hides are completely covered by the molten mass, the vacuum is stopped; it is preferred then to put the mass under pressure, exceeding 55 the atmospheric pressure.

It has been found, that by this manner the liquid will easily penetrate into the pores of the hides and fill them completely.

The present invention is also especially 60 valuable when used in connection with the process described in United States Patent No. 1,200,146 dated October 3, 1916, for the manufacture of leather products resembling leather, issued to Werner Spalteholz and 65 myself.

When hides are impregnated according to said process, the molten mass becomes enriched with benzene, or other liquid solvent as the case may be after each impregnation. 70 This benzene or other liquid solvent must be expelled from the molten mass by distillation with water vapors. However it is unavoidable, that after the distillation more or less water will remain in the molten 75 mass; this water however is of very injurious influence to the hides in some cases.

If on the contrary the hides, which are previously wholly dehydrated by a treatment with alcohol, acetone or their homologues, are impregnated with the molten mass by means of a vacuum and under following pressure, a reliable and complete impregnation is obtained. This is due to the known fact, that the previous dehydration 85 makes the hides considerably more resistant against elevated temperatures.

It is to be remarked, that without special precaution it is not possible to impregnate hides with this molten mass under pressure, 90 as it would be necessary to use temperatures, that would injure the hides under normal conditions.

Therefore the new process does not only 95 present the peculiar advantages of the known use of a vacuum in similar cases, but it allows in the first instance to dispense with the use of benzene and all other inflammable substances; besides the distillation with water vapors for the elimination 100 of the benzene is dispensed with and thereby the danger of injuring the hides by the remaining water is removed.

When I speak of alcohols I mean also to

include ketones and when I speak of hide I mean to include both hide and skin in the untanned state and leather.

Now what I claim and desire to secure by Letters Patent is the following:

- 5 1. The art of tanning hides comprising reducing the atmospheric pressure on the hides and then treating the hides while under reduced pressure with a molten asphaltic material, substantially as described.
- 10 2. The art of tanning hides comprising reducing the atmospheric pressure on the hides, treating the hides while under the reduced pressure with a molten asphaltic material and then subjecting said hides to a pressure exceeding atmospheric pressure.
- 15 3. The art of tanning hides comprising dehydrating hides by means of a substance having an attraction for water and impregnating the hides with filling substances while under a reduced pressure.
- 20 4. The art of tanning hides comprising dehydrating the hides by means of a suitable

substance having an attraction for water and impregnating the hides with a molten asphaltic material under reduced pressure.

5. The art of tanning hides comprising dehydrating the hides by means of an alcohol and impregnating the hides with asphaltum while under the reduced pressure.

6. The art of tanning hides comprising dehydrating the hides by means of a suitable liquid having an attraction for water, impregnating the hides with asphaltum while under the reduced pressure and then subjecting the hides to a pressure greater than atmospheric pressure.

That I claim the foregoing as my invention, I have signed my name in presence of two witnesses, this 26th day of January, 1916.

KURT HARING.

Witnesses:

JEAN GRUND,  
CARL GRUND.

Copies of this patent may be obtained for five cents each, by addressing the "Commissioner of Patents, Washington, D. C."